

## 1

2,794,388

## METHOD OF PREPARING A LITHOGRAPHIC PRINTING PLATE

Orson Warren Lake and Charles F. Amering, Rochester, N. Y., assignors to Eastman Kodak Company, Rochester, N. Y., a corporation of New Jersey

No Drawing. Application October 25, 1955,  
Serial No. 542,782

5 Claims. (Cl. 101—149.2)

This invention relates to lithography and particularly to a method for improving the ink receptivity of lithographic printing plates.

Lithographic printing plates have a hydrophilic surface which repels lithographic printing ink. In use, an image is formed on the surface of the plate which accepts ink and which prints the image in a lithographic printing press. Lithographic paper printing plates are usually coated with a mixture of a hardened hydrophilic organic colloid and an inert pigment. Suitable printing plates have a paper support which has been coated with a mixture of well hardened casein and a pigment such as clay, barium sulfate, etc. If the casein coated paper has a layer containing gelatin and pigment, it may be treated to render the surface less absorptive.

It is known that the ink receptive image can be formed photographically on a separate sheet and transferred to the lithographic printing plate. A process of this type is described in Clark and Cowden U. S. application Serial No. 267,482, filed January 21, 1952, now U. S. Patent No. 2,763,553. These processes have defects, however, mainly because the transferred image is not sufficiently durable in the printing operation and is not sufficiently ink receptive.

It is therefore an object of the present invention to provide a method for providing a lithographic printing plate having good ink receptivity and durability for printing. Other objects will appear from the following description of our invention.

These objects are accomplished by transferring an unhardened gelatin image to a lithographic printing plate which will repel greasy printing inks when wet with water, wetting the surface of the printing plate and the transferred gelatin image with a solution of tannic acid and thiourea after which the printing plate is wet with water and run in a lithographic printing press in the customary way.

A suitable paper printing plate has a melamine-formaldehyde sized paper stock of medium weight coated with a mixture of gelatin and baryta containing a gelatin hardening agent such as formaldehyde or aluminum chloride. A suitable plate may also be formed of a sized paper stock of medium weight rendered water repellent with a casein coating having about 0.15 to .6 g. of casein per square foot of surface. The casein coating may contain an inert pigment such as clay or baryta and may be treated, if desired, with a cuprammonium solution or a salt solution such as zinc acetate before, after or during application to the casein-pigment coat of a thin coating of a hydrophilic colloid such as sodium alginate, as described in U. S. Patent 2,534,650.

The photographic gelatin image which is to be transferred to the printing plate may be formed in various ways, but preferably is made and transferred as described in Yutzy and Yackel U. S. Patents 2,596,756 and 2,716,059. As described in these patents, a substantially unhardened gelatino-silver halide, which contains a tan-

## 2

ning developing agent or both a tanning and a non-tanning developing agent is exposed to a line or halftone image and developed to form a tanned or hardened gelatin image. The tanned gelatin image may also be formed by use of an external developing agent not incorporated in the emulsion layer. After a tanned or hardened gelatin image is formed in this way the remaining gelatin which is unhardened is transferred to an absorbent support, e. g. paper, cloth or wood, or in the present case, to the hydrophilic surface of a lithographic printing plate which will repel greasy printing inks when wet with water.

The gelatin image transferred in this way is soft and hydrophilic and must be rendered ink receptive as well as sufficiently hard and tough to withstand abrasion and printing on the lithographic press. We have found that this may be accomplished by treating the plate after the gelatin image has been transferred to it, with a solution containing tannic acid and thiourea and other agents if desired. In addition to tannic acid and thiourea, the solution used to treat the plate may contain ascorbic acid, aluminum chloride, sodium bisulfate, potassium bichromate, hydrochloric acid or chromic chloride.

The following examples illustrate our invention.

## Example 1

An image of a typewritten document was formed in a light-sensitive emulsion in the manner described in Yutzy and Yackel U. S. Patent 2,716,059 and the unhardened gelatin of the sensitive material was transferred to a lithographic printing plate instead of to a sheet of absorbent paper. A printing plate of the type described above was used, in this case a plate sold under the trade name Remington Rand Plastiplate. The transferred gelatin image was swabbed for 20 seconds with a solution of tannic acid and thiourea in water containing 10% tannic acid and 5% thiourea. The plate was heated for 20 seconds with light from two Photoflood lamps about one foot away and was then moistened with water or conventional lithographic etching solution, placed on an offset press and run under standard printing conditions. A run of 500 copies was obtained.

## Example 2

A typewritten document was exposed to the sensitive material described in Example 1 and the transfer made to a lithographic printing plate such as described above, in this case a plate sold under the trade name Polychrome V Kote Plate. The transferred image was swabbed with a solution in water of 4% tannic acid, 4% sodium bisulfate and 4% thiourea. The treated plate was then placed on an offset press and 100 to 150 copies were made in the usual way.

The use of thiourea in our formulas is particularly important since ink receptivity of the plate on the press is dependent on this material. The usual gelatin tanning agents are ineffective in the presence of thiourea but tannic acid is effective to harden the gelatin when thiourea is present.

One disadvantage of transferring the gelatin image from the matrix as described in Examples 1 and 2, to the lithographic plate is that certain plates cause the matrix to frill and transfer background gelatin, thus preventing satisfactory offset press results. This appears to be caused by the acidity of the surface of the offset plate which frequently has a surface pH of 4 to 5 whereas the matrix pH is about 9 to 11 at the time of transfer. However, matrix frill may be caused by high pigment-to-binder ratios in the surface coating of the master or inclusions of excessive amounts of gelatin reactors such as formaldehyde.

We have found that this undesirable frill may be

avoided by an alkaline surface treatment of the offset master, for example, by swabbing and drying it with an alkaline solution before making the transfer to the offset plate. This alkaline treatment does not affect the quality and life of the master on the offset press. Suitable alkaline solutions for this purpose are a 2% solution of borax or a 3% solution of sodium carbonate, ammonium hydroxide, sodium hydroxide, ethanolamine or methylamine. The following example illustrates this treatment.

*Example 3*

A lithographic printing plate such as described above, for example, a plate known as Quality Direct Image Plate sold by Polychrome Corporation of Yonkers, New York, or 7900 Series Plastiplate sold by Remington Rand Division of Sperry-Rand Corporation was hand rubbed with a 2% borax solution and dried. A transfer of a type-written image was then made to the plate as described in Example 1 and the plate was swabbed with the solution of tannic acid, sodium bisulfate and thiourea described in Example 2. The plate was then run on an offset press and at least 100 copies were obtained.

It will be understood that the examples and modifications described herein are illustrative only and that our invention is to be taken as limited only by the scope of the appended claims.

What we claim is:

1. The method of preparing a lithographic printing plate having good lithographic ink receptivity and durability, which comprises forming by exposure and development in a gelatino-silver halide emulsion layer of unhardened gelatin, a hardened gelatin image, transferring the unhardened gelatin portions of said emulsion layer to a lithographic printing plate which will repel greasy printing inks when wet with water, wetting the surface of the printing plate and the transferred gelatin image with a solution containing approximately 4% to 10% tannic acid and approximately 4% to 5% thiourea, and then wetting the surface of the printing plate with water and placing it on an offset printing press.

2. The method of preparing a lithographic printing plate having good lithographic ink receptivity and durability, which comprises forming by exposure and development in a gelatino-silver halide emulsion layer of unhardened gelatin, a hardened gelatin image, transfer-

ring the unhardened gelatin portions of said emulsion layer to a lithographic printing plate which will repel greasy printing inks when wet with water, wetting the surface of the printing plate and the transferred gelatin image with a solution containing approximately 4% to 10% tannic acid, approximately 4% to 5% thiourea and approximately 4% sodium bisulfate, and then wetting the surface of the printing plate with water and placing it on an offset printing press.

10 3. The method of preparing a lithographic printing plate having good lithographic ink receptivity and durability, which comprises forming by exposure and development in a gelatino-silver halide emulsion layer of unhardened gelatin, a hardened gelatin image, transferring the unhardened gelatin portions of said emulsion layer to a lithographic printing plate which will repel greasy printing inks when wet with water, wetting the surface of the printing plate and the transferred gelatin image with an aqueous solution containing 4% tannic acid, 4% thiourea and 4% sodium bisulfate, and then wetting the surface of the printing plate with water and placing it on an offset printing press.

15 4. The method of preparing a lithographic printing plate having good lithographic ink receptivity and durability, which comprises forming by exposure and development in a gelatino-silver halide emulsion layer of unhardened gelatin, a hardened gelatin image, washing the acidic surface of a lithographic printing plate which will repel greasy printing inks when wet with water, with an 20 alkaline solution to neutralize its acidity, transferring the unhardened gelatin portions of said emulsion layer to said printing plate, wetting the surface of the printing plate and the transferred gelatin image with an aqueous solution containing 4% tannic acid, 4% thiourea and 4% sodium bisulfate, and then wetting the surface of the printing plate with water and placing it on an offset printing press.

25 5. An aqueous solution for treating a lithographic printing plate having a gelatin image thereon, comprising approximately 4% to 10% tannic acid, approximately 4% to 5% thiourea and approximately 4% sodium bisulfate.

No references cited.